

# UNITED STATES PATENT OFFICE.

ARNOLD VON SOLEMACHER-ANTWEILER, OF SCHLOSS WACHENDORF, NEAR SATZVEY, GERMANY.

## ARTIFICIAL BUILDING-STONE.

SPECIFICATION forming part of Letters Patent No. 437,525, dated September 30, 1890.

Application filed March 29, 1890. Serial No. 345,879. (No specimens.)

*To all whom it may concern:*

Be it known that I, ARNOLD VON SOLEMACHER-ANTWEILER, chamberlain and lord of manor of Schloss Wachendorf, near Satzvey, in the Kingdom of Prussia and German Empire, have invented a new and useful Improved Method of Producing Weather-Proof Artificial Enamel Stones Indifferent Against Acids, of which the following is a specification.

This invention has reference to a new or improved manufacture of artistic enamel bricks and plates or tiles weather-proof, acid-proof, not penetrable by moisture, and of so highly durable a nature as to be practically indestructible. They are intended for use in building operations, whether to serve in lieu of ordinary facing-bricks, the same size as which they can be made, or to be employed alternately or in conjunction with ordinary facing-bricks—for example, in the adornment of facades. They are also intended to serve in the form of plates or tiles for covering walls in all cases where dryness, cleanliness, and elegance are desired, for which purposes it has been usual to employ known kinds of glazed clay plates or tiles of the less valuable or costly descriptions. My bricks, plates, or tiles are also specially suitable for use in the construction of friezes, floors, &c. They are opaque and can be produced as a pure white enamel, and also in all colors or shades of color and marbled, and with various patterns, designs, and emblems.

The enamel is made of a mixture of the following substances in or about the proportions stated, namely: one hundred parts, by weight, of silicic acid; five parts, by weight, of fluor-spar; five parts, by weight, of feldspar; twenty parts, by weight, of soda; five parts, by weight, of tin-ash; five parts, by weight, of alum-earth; five parts, by weight, of red lead; two and one-half parts, by weight, of talc; two and one-half parts, by weight, of cryolite, in a regenerative glass-melting furnace at a temperature of from about 1,500° to 2,000° and casting the resulting fluid mass, with eventual addition of suitable coloring agents, in molds into the form of bricks or plates or tiles of the desired shape and size with projecting border and interrupted transverse ribs or projections at the back.

In witness whereof I have hereunto set my hand in presence of two witnesses.

ARNOLD VON SOLEMACHER-ANTWEILER.

Witnesses:

F. H. THOMAS,  
D. J. PARTELLO.